

Feb. 16, 1932.

F. JORDAN

1,845,155

PROCESS FOR RAISING THE RESISTANCE OF ZINC TO TEARING DURING ROLLING

Filed July 30, 1928



Inventor:

F. Jordan

By: *Marks & Clark*  
Atty.s.

## UNITED STATES PATENT OFFICE

FRANZ JORDAN, OF WICKEDE-RUHR, GERMANY

## PROCESS FOR RAISING THE RESISTANCE OF ZINC TO TEARING DURING ROLLING

Application filed July 30, 1928, Serial No. 296,428, and in Germany June 12, 1928.

Hitherto the rolling of zinc sheet has been carried out in the heated condition and at a temperature amounting to about 100-150° C. Nevertheless, in spite of this heating, zinc 5 does not stand heavy rolling pressures since its power of resistance is only small and it tears easily under heavy rolling pressures or splits at the edges on being rolled.

Therefore, in order to reduce the amount 10 of waste, only small rolling pressures are employed at the present time and the blocks to be rolled are as thin and light in weight as possible. Then, when these blocks have been rolled down to a thickness of a few millimeters, this preliminary product is cut and the further rolling of the sheets takes place in so-called "packets" that is to say about ten to twenty plates are placed one on top of another and these are rolled down further in a 15 bundle under low pressure. In order that thickness of the sheet may be uniform the position of the separate plates must be changed at each rolling. This is termed "mixing" in practice.

20 It will be clear that the above described rolling process must proceed relatively slowly, and that waste always occurs. Rolling out of the material in band form has not been successfully accomplished because the roller pressure as hereinbefore explained, may not be sufficiently heavy.

The object of the present invention is to overcome these disadvantages.

The invention is based on the discovery 25 that a thin aluminium coating rolled on the zinc considerably increases the capability of the zinc for being rolled, so that heavy roller pressures can then be employed. There also results from this that the blocks to be rolled 30 may be of much thicker and heavier proportions than previously, which again must accelerate and cheapen the process to a very considerable extent.

The process is carried out in the following 35 manner. Zinc blocks of about 300-500 kg.

in weight and about 50-100 m. m. thick and of suitable width and length are plated in known manner on one or both sides with an aluminium coating, the thickness of which is about 5-10% the thickness of the core metal. 50 The plating is effected on a rolling apparatus to which the aluminium sheet is conducted from endless rollers on to the zinc block which is to be rolled, and the sheet is united to the zinc by pressure of the rollers. The 55 accompanying drawing shows the method by which the plating is carried out. Aluminium sheet 2 is supplied from rolls of the material 3, and is united to the surface of the zinc block 1 by pressing thereon by means of the 60 rollers 4. The further rolling of the plated blocks can then take place under heavy pressure in another suitable rolling machine. The aluminium coating prevents the zinc block 1 from tearing or from splitting to any 65 considerable extent at the edges. The capability of the zinc for being rolled and withstanding tearing is moreover completely changed owing to the coating, so that the 70 rolling process can take place without any considerable tearing or splitting occurring. It is also possible to roll out thin sheets of 75 any width in band form, since the heavy roller pressure automatically heats up the zinc to the degree necessary for the rolling process.

The aluminium coating also does not prevent the zinc sheet from being worked. For example, if the zinc is to be soft soldered, it 80 can easily be removed by scraping. On the other hand the resistance of the zinc to chemical or atmospheric attack is greatly increased by the aluminium coating. The new process therefore not only lessens the cost of manufacture of zinc sheets, but it can advantageously be employed in all cases in which the small resistance of the zinc to chemical action has hitherto been an obstacle to the 85 employment of zinc sheets.

What I claim is:—

A process for raising the resistance of zinc to tearing during rolling consisting in applying thin aluminium strips by pressure to a comparatively thick core of zinc so that the 5 aluminium strips completely cover the core on two opposite surfaces while the thickness thereof amounts to 5-10% of that of the core, subjecting these parts to a preliminary rolling process so as to effect a union thereof, and 10 finally rolling out this combined material into thin strips at high rolling pressures without intermediate heating so as to prevent cracking of the zinc core.

In testimony whereof I have signed my 15 name to this specification.

**FRANZ JORDAN.**

**20****25****30****35****40****45****50****55****60****65**